

## UNITED STATES PATENT OFFICE

1,958,136

METHOD OF SEASONING SHEETS CONTAIN-  
ING A SOLVENTGustavus J. Esselen, Swampscott, Mass., assignor  
to The Fiberloid Corporation, Indian Orchard,  
Mass., a corporation of MassachusettsNo Drawing. Application October 24, 1931,  
Serial No. 570,978

3 Claims. (Cl. 18—51)

The present application is a continuation in part of my former application, Serial No. 249,-744, filed January 26, 1928, for Method and apparatus for making a continuous web. In that application there is described a process of producing a continuous sheet or web of pyroxylin by extruding under pressure through an orifice a mix of pyroxylin containing a solvent such as an alcohol (either ethyl or methyl) or an ester such as ethyl acetate in the presence of camphor and setting the mix to form a self sustaining sheet by immersion in a bath of non-solvent liquid. By solvent I mean a liquid capable of forming with the other ingredients of the mix a colloidal solution; by non-solvent I mean a liquid which is incapable of forming such a solution.

My present invention is based on the discovery that the treatment described, when applied to unseasoned sheets formed by any suitable process, has the effect of seasoning them, i. e. removing the residue of solvent which persists tenaciously in them.

It is well recognized that sheets of pyroxylin or other cellulose ester whether made by the so-called cake process, i. e. by the formation of blocks or cylinders from which sheets are sliced or by some other process require long seasoning to reduce the residual amount of solvent contained in the sheets to the required minimum. This seasoning has ordinarily been accomplished preferably by hanging the sheets in hot rooms. Of necessity this process of seasoning is slow, ordinarily occupying a week or two according to the thickness of the sheet, its condition and the conditions of treatment, and is expensive because of the equipment required and of the large amount of stock which is processed.

I have discovered that certain liquids which are non-solvents of pyroxylin have the property of displacing solvents of pyroxylin from a sheet; and further that when the solvent has been displaced by the non-solvent, the non-solvent can be removed by evaporation much more rapidly than a solvent. For some reason unknown to me, pyroxylin appears to be much less tenacious of non-solvents than of solvents.

These discoveries have made possible an entirely new method of seasoning sheet pyroxylin which reduces the time required by many days.

Speaking generally, my process consists in immersing the unseasoned sheets containing a considerable percentage of a solvent of pyroxylin in a bath composed of a non-solvent which is capable of displacing the solvent, preferably, without

precipitating the pyroxylin, and then drying out the non-solvent. While a variety of liquids may be employed for the non-solvent bath the liquid must be one which is miscible with the solvent, if not in all proportions, then in certain proportions and under certain conditions. For instance, toluol in the aromatic series of hydrocarbons or carbon tetrachloride being completely miscible with ethyl or methyl alcohol may be employed as a non-solvent; or V. M. P. naphtha, so-called in the aliphatic series, which is miscible in certain but not in all proportions, may also be used. These non-solvents are capable of displacing the solvent without precipitating the pyroxylin. V. M. P. naphtha is commonly known as Varnish Makers' Petroleum and is characterized by the fact that it has a flash point not lower than 100° F. While its properties vary with the particular refining company, a typical sample shows a gravity of 47.6, an initial boiling point of 311° F., and an end point of 411° F.

In order to produce a seasoned sheet which is transparent, it is essential that the process of seasoning remove the excess solvent without precipitating the pyroxylin out of the solid solution. If the solution is precipitated, changes in physical properties occur, for instance, the stock becomes cloudy and brittle. Drying, which is the ordinary method of seasoning, removes the excess solvent without precipitating the pyroxylin. This result is accomplished more rapidly by the practice of the invention.

In practice I also find it desirable to use a sufficient quantity of the plasticizer employed in the pyroxylin to prevent any considerable extraction of the plasticizer from the pyroxylin sheet during treatment.

In practising my invention I make the sheet from a suitable mix containing nitrocellulose or the like; a solvent such as ethyl alcohol (containing if required a suitable denaturant) or methyl alcohol or ethyl acetate; camphor or other suitable plasticizer and any other ordinary ingredients employed in the manufacture of pyroxylin. The mix is then formed into sheets in whatever way chosen. Thereafter, I treat the sheets with a suitable non-solvent, for instance, a hydrocarbon of the aliphatic series. Suitable materials are naphtha of the grade known as V. M. P. naphtha, gasoline, toluol or carbon tetrachloride. These liquids have the property of dissolving camphor though they do not dissolve nitrocellulose and therefore tend to extract the camphor from the sheet, reducing the camphor content.

Accordingly, I use in the bath a sufficient amount of camphor and maintain the strength at such a point that the bath will not extract camphor from the sheet to a material extent.

5 As an example, a suitable bath is made of V. M. P. naphtha and camphor in the proportion of 66 parts of camphor by weight to 100 parts of naphtha. For sheets having a thickness of 0.020 inches an immersion for an hour or even less is 10 sufficient to extract or displace from the sheet the residual solvent, i. e. the alcohol remaining in the sheet at the time the sheet is formed. After removal from the bath the sheets are dried in any suitable manner as for instance by passing them 15 through a current of dry air. The time required for drying is relatively short and I find that the entire process of seasoning the sheet can be completed in less than eight hours instead of requiring a week as heretofore.

20 The herein described method embodying my invention produces a sheet having a surface which is at least as good as that of sheets produced by the methods heretofore employed and also results in the savings already described.

25

While I have described my invention as I practice it, in connection with the manufacture of pyroxylin sheets, I believe it to be applicable to sheets of other substances containing solvents.

I claim:

1. The process of seasoning a sheet of pyroxylin or the like containing alcohol which consists in treating the sheet with carbon tetrachloride to displace the alcohol and then drying out the carbon tetrachloride.

80 2. The process of seasoning a sheet of pyroxylin or the like containing alcohol, which consists in treating the sheet with V. M. P. naphtha to displace the alcohol and then drying out the V. M. P. naphtha.

85 3. The process of seasoning pyroxylin sheet material containing a solvent which consists in treating the sheet with a liquid selected from the group consisting of toluol, carbon tetrachloride, gasoline and V. M. P. naphtha to replace the solvent in the sheet, and then drying the sheet.

90 GUSTAVUS J. ESSELEN.

95

30

100

35

105

40

110

45

115

50

120

55

125

60

130

65

135

70

140

75

150